

## UNITED STATES PATENT OFFICE

2,160,375

WATER-REPELLENT TEXTILE MATERIAL  
AND PROCESS OF MANUFACTURING IT

Arthur Voss, Frankfort-on-the-Main-Hochst, and  
Hermann Staerk, Bad Soden in Taunus, Germany, assignors to I. G. Farbenindustrie Aktiengesellschaft, Frankfort-on-the-Main, Germany

No Drawing. Application December 31, 1936,  
Serial No. 118,678. In Germany January 4,  
1936

10 Claims. (Cl. 91—68)

This invention relates to water-repellent textile material and to a process of manufacturing the material and is a continuation in part of our application Ser. No. 94,482, filed August 5, 1936 and entitled "Water-repellent material and a process of manufacturing the material".

We have found that textile materials can be made water-repellent in an advantageous manner by treating them with solutions or emulsions of mixed polymerizates which are prepared from maleic anhydride the free acid or a functional derivative thereof and vinyl-esters of higher fatty acids (having at least 12 carbon atoms), for instance, according to the process described in U. S. Patent 2,047,398 for manufacturing mixed polymerisation products from maleic acid anhydrides and vinyl esters (see Example 4 of the U. S. Patent 2,047,398). These mixed polymerizates yield stable solutions or emulsions which, when applied to textile fibers, especially fibers of vegetable origin, such as, for instance, cotton, have a very good waterproofing action, the treated material being repellent to water to a very high extent. The material has this property directly after the treatment and does not require an after-treatment, as is the case in most similar processes.

With the same good result there may also be used the mixed polymerizate from maleic anhydride and the vinyl ether of an aliphatic alcohol of high molecular weight with at least 12 carbon atoms in the molecule, as free acid or a functional derivative thereof. These mixed polymerizates which as previously stated are obtainable according to the process described in U. S. Patent 2,047,398 (see Example 6 for the manufacture of mixed polymers from maleic acid anhydride and vinyl ethers) or which may be obtained by mutual polymerisation of a functional derivative of maleic acid and of a vinyl ester or vinyl ether of high molecular weight are composed of compounds of the formula:



wherein  $\text{R}_1$  and  $\text{R}_2$  stand for a member of the group consisting of  $\text{COOH}$ ,  $\text{COO}$ , alkyl,  $\text{CN}$ ,  $\text{CONH}_2$ .  $\text{R}_1$  and  $\text{R}_2$  together represent



and compounds of the formula



wherein  $\text{X}$  stands for  $\text{R}$ ,  $\text{OR}$  or  $\text{OOCR}$ ,  $\text{R}$  representing an aliphatic hydrocarbon radical with at least 12 carbon atoms.

The reaction upon the textile materials is executed in the following way: The textile material is introduced into the solution or emulsion of the mixed polymerizate and, after drying in the air, dried for a short time at a higher temperature (at about 100° C.).

The above described process is distinguished by the fact that the fiber is not only made waterproof when treated in this manner but that it retains its waterproofness even after repeated washing to an extent which could hitherto not be attained by any process, that is to say, the mixed polymerizates above characterized are so intimately combined with the fiber that similar to fast-dyestuffs, they irreversibly adhere to the fiber.

The following examples serve to illustrate the 20 invention but they are not intended to limit it thereto:

(1) A web of cotton or artificial silk is impregnated with a solution of 0.5 per cent strength of the mixed polymerizate from vinyl-octodecyl-ether and maleic-acid-dimethylester in carbon tetrachloride or a mixture thereof with alcohol, and is dried at ordinary temperature. The web thus treated has a very good water-repellent effect and does not lose this property even when 30 repeatedly washed or boiled with water.

(2) Loose wool is impregnated as indicated in Example 1 with a solution of the mixed polymerizate from vinyl-octodecyl-ether and maleic acid in a mixture consisting of methylene chloride and ethyl-alcohol. After drying, the wool thus treated shows an enhanced water-repelling effect which it does not lose by washing.

(3) A web of cotton or artificial silk is impregnated with a solution in methylene chloride 40 of the mixed polymerizate from vinyl-stearate and the semi-ester of maleic acid with methyl alcohol, and is dried at ordinary temperature. The fabric thus treated has a very good water-repellent effect and does not lose this property 45 even after repeated washing or boiling with water.

(4) A web of viscose artificial silk is treated with a solution of 0.5% strength in alcohol and carbon tetrachloride of the mixed polymerizate from maleic acid and vinyl-octodecyl-ether obtained by treating with steam the anhydride mixed polymerizate and dried for a short time. The fabric thus treated has a very good water- 55

repellent effect and does not lose this property even by washing or boiling.

(5) Loose spun rayon is impregnated with a solution of 2% strength in carbon tetrachloride of the mixed polymerisate from vinyl-stearate and maleic acid monomethyl ester, squeezed and dried. The spun rayon thus treated is very hydrophobe and does not lose this property by subsequent fulling.

(6) Piece goods consisting of a mixture of wool and spun rayon are impregnated with an aqueous solution of 1% strength of the pyridine salt of a mixed polymerisate from maleic acid and vinyl-hexadecyl ether and subjected for a short time to a heat treatment at 90° C.-100° C. The material thus treated has a very good water-repellent effect and does not lose this property even by washing.

(7) Loose cotton is impregnated with an aqueous solution of 0.8% strength of the amide-ammonium salt of the mixed polymerisate from maleic acid and vinyl stearate, obtainable by the treatment of the anhydride with dry ammonia, and dried. Cotton thus treated has the same properties as those of the material obtained according to Example 6.

(8) A cotton fabric is impregnated by passage through a solution of a mixed polymerisate from vinyl stearate and maleic anhydride in methylene chloride, dried by exposure to air and heated for half-an-hour to about 100° C. The fabric thus treated is highly repellent to water and does not lose the property even after repeated washing with water and soap.

(9) A cotton or artificial silk fabric is impregnated with an aqueous emulsion of a mixed polymerisate from vinyl palmitate and maleic anhydride and worked up as indicated in Example 8. If desired the heat-treatment may be followed by a further treatment with aluminium formate, whereby the water-repelling effect is further increased. This fabric also retains its water-repellent property after repeated washing.

(10) Loose wool is immersed into a solution of 5 per cent strength of a mixed polymerisate from vinyl stearate and maleic anhydride, pressed and dried at 90-100° C. The material thus treated has an increased resistance to water.

(11) A fabric of cotton or artificial silk is impregnated with a solution of a mixed polymerisate from vinyl octo-decyl ether and maleic anhydride in ethylene chloride, dried and then heated for a short time at about 100° C., whereby the mixed polymerisate is intimately combined with the fibre. The fabric thus treated is highly repellent to water and does not lose this property even when washed with water and soap.

Instead of the aforesaid mixed polymerisate from maleic anhydride and vinyl octodecyl ether, the mixed polymerisate from maleic anhydride and the vinyl ether of the alcohol mixture obtainable by reduction of the coconut oil fatty acid and which contains chiefly carbon chains with 12 to 14 carbon atoms, may be applied in a similar manner for rendering the textile fiber highly waterproof.

(12) A cotton fabric is impregnated with a solution of 0.5% strength of a mixed polymerisate of maleic anhydride and vinyl dodecyl ether in carbon tetrachloride and dried subsequently, finally for a short time at a temperature of 100° C. The fabric treated in this manner is highly repellent to water and does not lose this property even when washed with water and soap.

(13) A fabric of viscose artificial silk is im-

pregnated with a solution of 0.2 per cent strength of a mixed polymerisate of maleic anhydride and the vinyl-ether of the montan wax alcohol of the formula  $C_{27}H_{55}C(C_2H_5)_2OH$  in methylene-chloride. After drying which is finally performed for a short time at a temperature of 100° C., this artificial silk shows an extraordinarily good water-repellent effect, and does not lose this property when extracted with organic solvents or boiled or washed with water.

(14) Loose wool is impregnated with a solution of 0.5 per cent strength of a mixed polymerisate of maleic anhydride and hexa-decylene in carbon tetrachloride. The material thus treated shows after drying which is finally performed for a short time at a temperature of 100° C., an excellent water-repellent effect and a great stability to water.

We claim:

1. A process for waterproofing textile materials which comprises treating the textile materials with baths containing mixed polymerisates being composed of compounds of the formula:



$R_1$  and  $R_2$  standing for a member of the group consisting of  $COOH$ ,  $COO$ , alkyl,  $CN$  and  $CONH_2$  and  $R_1$  and  $R_2$  together stand for



and compounds of the formula:



wherein  $X$  stands for a member of the group consisting of  $R$ ,  $OR$ ,  $OOC.R$ ,  $R$  standing for an aliphatic hydrocarbon radical with at least 12 carbon atoms.

2. A process for waterproofing textile materials which comprises treating the textile materials with baths containing mixed polymerisates being composed of maleic acid of the formula:



and compounds of the formula:



wherein  $X$  stands for a member of the group consisting of  $R$ ,  $OR$ ,  $OOC.R$ ,  $R$  standing for an aliphatic hydrocarbon radical with at least 12 carbon atoms.

3. A process for waterproofing textile materials which comprises treating the textile materials with baths containing mixed polymerisates being composed of maleic acid of the formula:



and vinyloctodecylether.

4. A process for waterproofing textile materials which comprises treating the textile materials with baths containing mixed polymerisates being composed of maleic acid of the formula:



and vinylhexadecylether.

5. Textile materials impregnated with mixed polymerisates being composed of compounds of the formula:



$R_1$  and  $R_2$  standing for a member of the group

consisting of COOH, COO, alkyl, CN, and CONH<sub>2</sub> and R<sub>1</sub> and R<sub>2</sub> together stand for



and compounds of the formula:



10. wherein X stands for a member of the group consisting of R, OR, O.CO.R, R standing for an aliphatic hydrocarbon radical with at least 12 carbon atoms.

6. Textile materials impregnated with mixed polymerisates being composed of maleic acid of the formula



and compounds of the formula:



wherein X stands for a member of the group consisting of R, OR, O.OCR, R standing for an aliphatic hydrocarbon radical with at least 12 carbon atoms.

7. Textile materials impregnated with mixed polymerisates being composed of maleic acid of the formula:



and vinyloctodecylether.

8. Textile materials impregnated with mixed polymerisates being composed of maleic acid of the formula:



and vinylhexadecylether.

9. A process of waterproofing textile materials which comprises treating the textile materials with baths containing mixed polymerizates from maleic anhydride and the compound of the formula H<sub>2</sub>C=CH.O.C<sub>12</sub>H<sub>25</sub>.

10. Textile materials impregnated with mixed polymerizates from maleic anhydride and the compound of the formula



ARTHUR VOSS.

HERMANN STÄRK.

25

CERTIFICATE OF CORRECTION.

Patent No. 2,160,375.

ARTHUR VOSS, ET AL.

May 30, 1939.

It is hereby certified that error appears in the printed specification of the above numbered patent requiring correction as follows: Page 1, first column, line 46, and page 3, first column, line 1, claim 5, strike out the comma after "COO" and insert instead a period; page 1, first column, line 47, strike out the period after "CONH<sub>2</sub>" and insert instead a comma; page 2, second column, line 27, claim 1, strike out the comma after "COO"; and that the said Letters Patent should be read with this correction therein that the same may conform to the record of the case in the Patent Office.

Signed and sealed this 19th day of September, A. D. 1939.

Henry Van Arsdale,

Acting Commissioner of Patents.

(Seal)

consisting of COOH, COO, alkyl, CN, and CONH<sub>2</sub> and R<sub>1</sub> and R<sub>2</sub> together stand for



and compounds of the formula:



10. wherein X stands for a member of the group consisting of R, OR, O.CO.R, R standing for an aliphatic hydrocarbon radical with at least 12 carbon atoms.

6. Textile materials impregnated with mixed polymerisates being composed of maleic acid of the formula



and compounds of the formula:



wherein X stands for a member of the group consisting of R, OR, O.OCR, R standing for an aliphatic hydrocarbon radical with at least 12 carbon atoms.

7. Textile materials impregnated with mixed polymerisates being composed of maleic acid of the formula:



and vinyloctodecylether.

8. Textile materials impregnated with mixed polymerisates being composed of maleic acid of the formula:



and vinylhexadecylether.

9. A process of waterproofing textile materials which comprises treating the textile materials with baths containing mixed polymerizates from maleic anhydride and the compound of the formula H<sub>2</sub>C=CH.O.C<sub>12</sub>H<sub>25</sub>.

10. Textile materials impregnated with mixed polymerizates from maleic anhydride and the compound of the formula



ARTHUR VOSS.

HERMANN STÄRK.

25

CERTIFICATE OF CORRECTION.

Patent No. 2,160,375.

ARTHUR VOSS, ET AL.

May 30, 1939.

It is hereby certified that error appears in the printed specification of the above numbered patent requiring correction as follows: Page 1, first column, line 46, and page 3, first column, line 1, claim 5, strike out the comma after "COO" and insert instead a period; page 1, first column, line 47, strike out the period after "CONH<sub>2</sub>" and insert instead a comma; page 2, second column, line 27, claim 1, strike out the comma after "COO"; and that the said Letters Patent should be read with this correction therein that the same may conform to the record of the case in the Patent Office.

Signed and sealed this 19th day of September, A. D. 1939.

Henry Van Arsdale,

Acting Commissioner of Patents.

(Seal)